

## UNITED STATES PATENT OFFICE

2,237,011

## SIMULTANEOUS PRODUCTION OF MAGNESIUM AND LOW CARBON FERROALLOYS

Ernst A. Pokorny, London, England, assignor to  
"Electrometal" Societe Anonyme, of LuxembourgNo Drawing. Application November 13, 1939,  
Serial No. 304,153

4 Claims. (Cl. 75—67)

It is known that the oxyde of magnesium can be reduced by silicon or carbon or else by compounds of silicon or carbon such as silicides or carbides respectively under conditions to yield metallic magnesium. The reaction requires temperatures of more than 1200 centigrades and must take place in vacuum or in a reducing atmosphere.

Under these conditions of working the question of apparatus and the building material used is very difficult to solve.

When working in the molten state, temperatures of more than 1700 centigrades are required for melting and even then the degree of liquidity obtained is not yet satisfactory for continuous technical working, because the slags containing oxyde of magnesium are, it is known, hard to liquefy.

On the other hand, when working in a sphere of temperatures at which the reacting materials are not yet molten, the reaction requires still temperatures of at least 1250 centigrades. As the reacting materials must not come into contact with the combustion gases, but, on the other hand, internal heating by metallic or carbon resistance is not applicable because the heaters are destroyed by the metallic vapors, it is necessary to work in enclosed reaction chambers heated from outside. This, however, puts a maximum strain on the constructing materials in question, so that the wear of the apparatus is very great, which in turn greatly increases the production cost by repairs required.

In order to render the process economical it is, therefore, necessary to modify it in a manner that by-products of high value can be obtained, the utilisation of which covers part of the cost.

Object of the present application is a process which allows the simultaneous production of magnesium metal and ferroalloys, low in carbon, as for instance: ferro-chromium, ferro-manganese etc. It has been ascertained by thorough experiments that neither manganese nor chromium react with the oxyde of magnesium at the temperature in question. Thus the reduction of the oxyde of magnesium by silicon, as such known, can be carried out in a manner that allows the utilisation of alloys of ferro-chromium-silicon, ferro-manganese-silicon etc. as reducing agents. It is known that carbon in alloys of ferro-chromium and ferro-manganese is displaced by silicon so f. i. an alloy containing about 30% of silicon does not contain more than, at most, 0.5% of carbon. The same is true in the case of ferro-manganese.

The working process of utilisation of ferro-chromium-silicon or ferro-manganese-silicon as reducing agents is as follows: oxyde of magnesium or materials containing oxyde of magnesium (f. i. dolomite), powdered or well granulated are thoroughly mixed with ferro-chromium-silicon or ferro-manganese-silicon containing about 30—45% of silicon (the latter equally well powdered). It is advisable to add quick lime if the raw-material does not contain lime in a sufficient quantity or any at all. The mixture, either loose or briquetted, is heated in a stream of hydrogen or of an inert gas or in vacuum up to a temperature of 1250 to 1350 centigrades.

15. This process is performed in a tube- or muffle-furnace, heated from outside, which may also be constructed as a rotary furnace. Alternatively the furnace can also be an electric arc- or tube- or muffle-furnace fitted with electrical internal heaters (graphite or carbon resistance).

20. As soon as the reaction is finished and the magnesium-metal-vapours formed, have been removed from the reaction chamber or have condensed in it, the residue is removed from the furnace and is molten by adding suitable fluxes in an electric furnace, the slags formed are poured away after having separated from metal, and the metal, still containing some percent of silicon is refined as required. The ferro-chromium or ferro-manganese of low carbon and silicon contents thus obtained represents a marketable product of high value.

25. The reduction of the oxyde of magnesium by silicon can be carried out also in an electric arc furnace allowing to heat the mixture by radiating heat up to the temperature of reduction. In this case, after the reduction has been completed, the residue of the reaction is heated directly by means of the arc, adding fluxes such as silica, fluorspar etc. if necessary. The residue melts and by this the ferro-chromium or the ferro-manganese is separated from the slags.

30. The process may also be carried out in a high frequency furnace working with the silicon containing ferroalloy in a molten state.

35. Instead of ferro-chromium-silicon or ferro-manganese-silicon also other alloys may be used in the same manner.

40. The residue of the reaction can be subjected to a mechanical or electromagnetic process of separation in order to obtain the ferroalloy separate from the other components.

45. Having now particularly described and ascertained the nature of the said invention and in

what manner the same is to be performed I declare that what I claim is:

1. A process for the recovery of a binary ferro-alloy and of magnesium from a ternary ferro-silicon alloy and a magnesia containing material which process comprises the steps of reacting the magnesia containing material with a ternary ferro-silicon alloy selected from the group consisting of ferro-manganese-silicon and ferro-chromium-silicon, and removing the magnesium, 10 and separating the binary ferroalloy from the silica containing slag.

2. A process as claimed in claim 1, in which the

magnesia containing material and the ternary ferro silicon are reacted with one another by heating a mixture of these materials in the absence of atmospheric oxygen to a temperature between 1250° and 1350° C.

3. A process as claimed in claim 1 in which the magnesium is removed from the reaction mixture by vaporization and subsequent condensation.

4. A process as claimed in claim 1 in which the binary ferroalloy is separated from the silica containing slag with the aid of heat and a flux.

ERNST A. POKORNY.